

## UNITED STATES PATENT OFFICE

2,435,525

## ELECTRODEPOSITION OF SILVER FROM A HIGH SILVER CYANIDE CONTENT BATH

Joseph S. Williams, New Augusta, and Walter R. Binai, Indianapolis, Ind., assignors to P. R. Mallory & Co., Inc., Indianapolis, Ind., a corporation of Delaware

No Drawing. Application May 5, 1942,  
Serial No. 441,866

9 Claims. (Cl. 204—46)

1

This invention relates to silver plating.

An object of the invention is to improve silver electrodeposition processes, the plating baths used in such processes and the product of such processes.

Another object is to produce smooth and bright silver deposits of substantial thickness by a process capable of use on a large production scale.

A further object is to produce silver electrodeposits suitable for use as bearing surfaces in internal combustion engines and the like.

Other objects of the invention will be apparent from the following description taken in connection with the appended claims.

The present invention comprises the combination of elements, methods of manufacture, and the product thereof brought out and exemplified in the disclosure hereinafter set forth, the scope of the invention being indicated in the appended claims.

While a preferred embodiment of the invention is described herein, it is contemplated that considerable variation may be made in the method of procedure and the combination of elements without departing from the spirit of the invention.

This invention relates to silver electrodeposits and means for obtaining them and particularly to the thicker types of deposits such as are suitable for bi-metals, inlays, overlays, silver lined bearings, electric contacts, commutators, slip rings and other types of silver deposits. We have found that silver plated steel shells made according to the present invention can be used successfully for bearings for airplane engines. The silver can also be deposited in the form of inlays in copper base backings for use as electric contacts.

It has generally been recognized in the past that the use of higher concentrations of silver cyanide, potassium carbonate and free cyanide and an increase of temperature permits silver plating at higher current densities. Agitation of the plating solution also makes possible increased plating speeds.

Since higher current densities permit more rapid production it may be assumed that electroplaters have heretofore used the highest current densities which they have found to be consistent

2

with good results. The usual current densities used for silver plating in the past have been in the order of 3 to 7 amperes per square foot, a density of 10 amperes being considered very high.

5 More recently experiments have been made with higher current densities for extremely thin silver coatings but, so far as we are aware, current densities substantially above those mentioned have not heretofore been found practicable for deposits of substantial thickness.

We have discovered that by departing radically from the values of plating bath concentrations and current densities used heretofore and by using values of a much higher order of magnitude, we have been able to produce smooth and bright silver deposits of substantial thickness on a mass production scale. The quality of the silver deposits we have been able to obtain is, in fact, of such a high degree as to permit their 10 use for aircraft engine bearings.

The process of the present invention can be used for applying silver deposits to various bases such as copper, iron and their alloys, for example.

The plating of steel bearing shells will be described below by way of example.

As smooth a finish as possible should be obtained by machining or grinding the surface of the steel shell which is to receive the silver deposit. The article to be plated is degreased and then electrolytically cleaned in an alkaline cleaning solution. After removal it is desirable to 15 thoroughly rinse the article in water.

Before silver plating it is desirable to apply a copper strike in a copper cyanide bath followed by a rinse and a dip in cyanide solution free of copper and silver. A silver strike is then immediately applied before the surface has a chance to dry.

## Silver strike bath

|                                                                                                                                             | Grams per liter |
|---------------------------------------------------------------------------------------------------------------------------------------------|-----------------|
| Silver cyanide                                                                                                                              | 2.0 to 2.75     |
| Free potassium cyanide                                                                                                                      | 150 to 180      |
| Potassium carbonate                                                                                                                         | 15 to 20        |
| 45 A current density of 30 amperes per square foot for 20 seconds may be used for the silver strike with a bath temperature of 90 to 95° F. |                 |
| 50 After the silver strike the surface should appear bright and uniform. The article is immediately transferred to the silver plating bath. |                 |

## Silver plating bath

|                        | Grams per liter |
|------------------------|-----------------|
| Silver cyanide         | 105 to 115      |
| Free potassium cyanide | 140 to 150      |
| Potassium carbonate    | 65 to 70        |
| Potassium hydroxide    | 2 to 5          |

A carbon disulphide brightener is used in the form of potassium cyanide solution which has been allowed to stand in contact with carbon disulphide. One or two c. c. per gallon are added to the plating bath as required. Other brighteners, such as sodium thiosulphate may be substituted, if desired.

The pH of the plating bath will normally fall between 12.6 and 13.4.

Plating is effected with a current density of 30 amperes per square foot of cathode surface if rocker arm agitation of the solution is used. With circulation of the solution the current can be increased to between 45 and 250 amperes per square foot. Under these conditions the circulation should be such as to produce a flow of 30 to 40 linear feet of solution per minute past the surface being plated.

The bath should preferably be kept at a temperature of 118 to 122° F. during plating.

While the above are the preferred conditions, given by way of example, it is contemplated that some deviation from these conditions can be made in some instances. Thus the silver plating bath may contain:

Silver cyanide in excess of 90 grams per liter. Free potassium cyanide, from 20% to 150% of the amount of silver cyanide.

Potassium carbonate, from a trace up to 80 grams per liter.

Potassium hydroxide, 2 to 5 grams per liter to bring the pH between 12.6 and 13.4.

Sodium cyanide may be substituted for the potassium cyanide in equal molecular proportions, although the potassium salt is preferred.

It will be noted that the silver content we use is much higher than that used by the prior art as well as the amount of free cyanide. However, the potassium carbonate is proportionally smaller in relation to the other ingredients.

The temperatures used should be kept between a minimum of 105° F. and a maximum of 120° F., preferably not in excess of 122° F. with carbon disulphide brightener. With sodium thiosulphate brightener the temperatures as high as 130° F. may be used. These plating temperatures are well above those heretofore followed by the art.

The current densities used may be between 30 and 250 amperes per square foot, the agitation of the solution being increased for the higher densities.

While the present invention, as to its objects and advantages, has been described herein as carried out in specific embodiments thereof, it is not desired to be limited thereby but it is intended to cover the invention broadly within the spirit and scope of the appended claims.

What is claimed is:

1. The method of making smooth and bright deposits of silver of substantial thickness which comprises electrodepositing the silver from a plating bath containing 90 to 115 grams per liter of silver cyanide, potassium carbonate in amounts from a trace to 80 grams per liter, and potassium hydroxide sufficient to bring the pH between 12.6 and 13.4 at a current density of at

least 30 amperes per square foot of the surface to be plated.

2. The method of making smooth and bright deposits of silver of substantial thickness which comprises electrodepositing the silver from a plating bath containing 90 to 115 grams per liter of silver cyanide, free potassium cyanide of 20% to 150% of the amount of silver cyanide, potassium carbonate in amounts from a trace to 80 grams per liter, and potassium hydroxide sufficient to bring the pH between 12.6 and 13.4 using a current density of at least 30 amperes per square foot of the surface area to be plated.

3. The method of making smooth and bright deposits of silver of substantial thickness which comprises electrodepositing the silver from a plating bath containing 90 to 115 grams per liter of silver cyanide, free potassium cyanide of 20% to 150% of the amount of silver cyanide in the bath, potassium carbonate in amounts from a trace to 80 grams per liter, and potassium hydroxide sufficient to bring the pH between 12.6 and 13.4 using a current density of at least 30 amperes per square foot of the surface area to be plated and maintaining the plating bath at a temperature between 105° and 130° F.

4. The method of making smooth and bright deposits of silver of substantial thickness which comprises electrodepositing the silver from a plating bath containing silver cyanide 90 to 115 grams per liter, free potassium cyanide between 20% and 150% of the amount of silver cyanide in the bath, potassium carbonate from a trace to 80 grams per liter, and potassium hydroxide sufficient to bring the pH between 12.6 and 13.4 using a current density of between 30 and 250 amperes per square foot of the surface to be plated, the bath being agitated meanwhile.

5. The method of making smooth and bright deposits of silver of substantial thickness which comprises electrodepositing the silver from a plating bath containing silver cyanide 90 to 115 grams per liter, free potassium cyanide between 20% and 150% of the amount of silver cyanide in the bath, potassium carbonate from a trace to 80 grams per liter, and potassium hydroxide sufficient to bring the pH between 12.6 and 13.4 using a current density of between 30 and 250 amperes per square foot of the surface to be plated, the bath being maintained at a temperature between 105° and 130° F. and agitated meanwhile.

6. The method of making smooth and bright deposits of silver of substantial thickness which comprises electrodepositing the silver from a plating bath containing silver cyanide between 105 to 115 grams per liter, free potassium cyanide between 140 to 150 grams per liter, potassium carbonate between 65 to 70 grams per liter, and potassium hydroxide sufficient to bring the pH between 12.6 and 13.4 using a current density of between 30 to 60 amperes per square foot of the surface to be plated, the bath being agitated meanwhile.

7. The method of making smooth and bright deposits of silver of substantial thickness which comprises electrodepositing the silver from a plating bath containing silver cyanide between 105 to 115 grams per liter, free potassium cyanide between 140 to 150 grams per liter, potassium carbonate between 65 to 70 grams per liter, and potassium hydroxide sufficient to bring the pH between 12.6 and 13.4 using a current density of between 30 to 60 amperes per square foot of the surface to be plated, the bath being maintained

at a temperature between 118° and 122° F. and agitated meanwhile.

8. A plating bath for high current density electrodeposition of silver, said bath containing—

Silver cyanide, 90 to 115 grams per liter;

Free potassium cyanide, from 20% to 150% of the amount of silver cyanide;

Potassium carbonate, from a trace to 80 grams per liter;

Potassium hydroxide sufficient to bring pH between 12.6 and 13.4.

9. A plating bath for high current density electrodeposition of silver, said bath containing—

Silver cyanide, 105 to 115 grams per liter;

Free potassium cyanide, 140 to 150 grams per liter;

Potassium carbonate, 65 to 70 grams per liter;

Potassium hydroxide, 2 to 5 grams per liter.

JOSEPH S. WILLIAMS.

WALTER R. BINAI.

#### REFERENCES CITED

10 The following references are of record in the file of this patent:

Transactions of the Electrochemical Society: vol. LIX, pp. 303-305 (1931); vol. 80, pp. 464, 467, 474 (1941).

15 Metal Industry, Nisol, pp. 275-277, Mar. 22, 1940.